



US006864028B1

(12) **United States Patent**  
**Jubran et al.**

(10) **Patent No.:** **US 6,864,028 B1**  
(b5) **Date of Patent:** **Mar. 8, 2005**

(54) **DI-HYDRAZONE BASED CHARGE  
TRANSPORT COMPOUNDS**

(75) Inventors: **Nusrallah Jubran**, St. Paul, MN (US); **Zbigniew Tokarski**, Woodbury, MN (US); **Kam W. Law**, Woodbury, MN (US); **Evaldas Burbulis**, Kaunas (LT); **Vaida Andruleviciute**, Kaunas (LT)

(73) Assignee: **Samsung Electronics Co., Ltd.**, Suwon (KR)

(\*) Notice: Subject to any disclaimer, the term of this patent is extended or adjusted under 35 U.S.C. 154(b) by 174 days.

(21) Appl. No.: **10/396,204**

(22) Filed: **Mar. 25, 2003**

**Related U.S. Application Data**

(60) Provisional application No. 60/368,255, filed on Mar. 28, 2002.

(51) **Int. Cl.**<sup>7</sup> ..... **G03G 5/047**; G07D 209/82

(52) **U.S. Cl.** ..... **430/73**; 430/78; 430/79; 430/58.35; 399/159; 546/95; 546/96; 548/444; 564/251

(58) **Field of Search** ..... 430/73, 78, 79, 430/58.35; 399/159; 546/95, 96; 548/444; 564/251

(56) **References Cited**

**U.S. PATENT DOCUMENTS**

|                 |         |                           |
|-----------------|---------|---------------------------|
| 4,297,426 A     | 10/1981 | Sakai et al.              |
| 4,476,137 A     | 10/1984 | Haviv et al.              |
| 4,786,571 A     | 11/1988 | Ueda                      |
| 4,957,838 A     | 9/1990  | Aruga et al.              |
| 5,128,227 A     | 7/1992  | Monbaliu et al.           |
| 5,274,116 A     | 12/1993 | Martin et al.             |
| 5,932,384 A     | 8/1999  | Mitsumori et al.          |
| 6,001,522 A     | 12/1999 | Woo et al.                |
| 6,020,096 A     | 2/2000  | Fuller et al.             |
| 6,030,734 A     | 2/2000  | Mitsumori                 |
| 6,066,426 A     | 5/2000  | Mott et al.               |
| 6,099,996 A     | 8/2000  | Yanus et al.              |
| 6,140,004 A     | 10/2000 | Mott et al.               |
| 6,214,503 B1    | 4/2001  | Gaidelis et al.           |
| 6,689,523 B2 *  | 2/2004  | Law et al. .... 430/58.35 |
| 6,696,209 B2 *  | 2/2004  | Law et al. .... 430/58.35 |
| 2003/0104294 A1 | 6/2003  | Law et al.                |
| 2003/0113132 A1 | 6/2003  | Law et al.                |
| 2003/0113643 A1 | 6/2003  | Law et al.                |
| 2003/0113644 A1 | 6/2003  | Law et al.                |
| 2003/0129513 A1 | 7/2003  | Jubran et al.             |
| 2003/0138712 A1 | 7/2003  | Law et al.                |
| 2003/0198880 A1 | 10/2003 | Law et al.                |

**FOREIGN PATENT DOCUMENTS**

GB 1047525 11/1966

**OTHER PUBLICATIONS**

Frank R. Atherton and Robert W. Lambert, *Synthesis of 3(S)-Acylamino-1-[ (Phenyl)(1H-Tetrazol-5-YL)Amino]-2-Azetidinones*, Symposia-in-Part Number 10: Recent Aspects of the Chemistry of E-Lactams, 1983, vol. 39, No. 15., pp. 2599-2608.

G. V. Boyd and S. R. Dando, *The Dimerisation of 5-Methylene- $\alpha$ -2-1,3,4-oxadiazolines*, Journal of The Chemical Society, 1971.

Yasuoki Murakami, Yuusaku Yokoyama, Chiyoko Sasakura, and Makiko Tamagawa, *An Efficient Synthesis of 1,1-Disubstituted Hydrazines*, Chemical & Pharmaceutical Bulletin, Feb. 1983, vol. 31, No. 2, pp. 423-428.

\* cited by examiner

**Primary Examiner**—Mark A. Chapman

(74) **Attorney, Agent, or Firm**—Patterson, Thuente, Skaar & Christensen, P.A.

(57) **ABSTRACT**

Improved organophotoreceptors have:

(a) a charge transport compound having the formula



where  $\text{R}_1$  and  $\text{R}_2$  are, independently, an (N,N-disubstituted) arylamine group, such as a julolidine group, a triphenyl amine group, or an N-substituted carbazole group;

$\text{R}_3$  and  $\text{R}_4$  are, independently, an alkylsulfonylphenyl group; and

$\text{X}$  is a linking group having the formula  $-(\text{CH}_2)_m-$ , branched or linear, where  $m$  is an integer between 0 and 20, inclusive, and one or more of the methylene groups is optionally replaced by an oxygen atom, a carbonyl group, urethane, urea, an ester group, a  $-\text{NR}_5$  group, a  $\text{CHR}_6$  group, or a  $\text{CR}_7\text{R}_8$  group where  $\text{R}_5$ ,  $\text{R}_6$ ,  $\text{R}_7$ , and  $\text{R}_8$  are, independently, H, an alkyl group, or aryl group;

(b) a charge generating compound; and

(c) an electrically conductive substrate over which the charge transport compound and the charge generating compound are located.

**18 Claims, No Drawings**

## 1

DI-HYDRAZONE BASED CHARGE  
TRANSPORT COMPOUNDSCROSS REFERENCE TO RELATED  
APPLICATIONS

The application claims priority to U.S. Provisional Patent Application Ser. No. 60/368,255 filed Mar. 28, 2002 to Law et al., entitled "Electrophotographic Organophotoreceptors With Novel Charge Transport Compounds," incorporated herein by reference.

## FIELD OF INVENTION

This invention relates to organophotoreceptors suitable for use in electrophotography and, more specifically, to flexible organophotoreceptors having charge transport compounds comprising two sulfonylphenylhydrazones groups.

## BACKGROUND

In electrophotography, an organophotoreceptor in the form of a plate, disk, sheet, belt, drum or the like having an electrically insulating photoconductive element on an electrically conductive substrate is imaged by first uniformly electrostatically charging the surface of the photoconductive layer, and then exposing the charged surface to a pattern of light. The light exposure selectively dissipates the charge in the illuminated areas, thereby forming a pattern of charged and uncharged areas. A liquid or solid toner is then deposited in either the charged or uncharged areas depending on the properties of the toner to create a toned image on the surface of the photoconductive layer. The resulting toned image can be transferred to a suitable receiving surface such as paper. The imaging process can be repeated many times to complete a single image and/or to reproduce additional images.

Both single layer and multilayer photoconductive elements have been used. In single layer embodiments, a charge transport material and charge generating material are combined with a polymeric binder and then deposited on the electrically conductive substrate. In multilayer embodiments, the charge transport material and charge generating material are in the form of separate layers, each of which can optionally be combined with a polymeric binder, deposited on the electrically conductive substrate. Two arrangements are possible. In one arrangement (the "dual layer" arrangement), the charge generating layer is deposited on the electrically conductive substrate and the charge transport layer is deposited on top of the charge generating layer. In an alternate arrangement (the "inverted dual layer" arrangement), the order of the charge transport layer and charge generating layer is reversed.

In both the single and multilayer photoconductive elements, the purpose of the charge generating material is to generate charge carriers (i.e., holes and/or electrons) upon exposure to light. The purpose of the charge transport compound is to accept at least one type of these charge carriers, generally holes, and transport them through the charge transport layer in order to facilitate discharge of a surface charge on the photoconductive element.

## SUMMARY OF THE INVENTION

In a first aspect, the invention features an organophotoreceptor that includes:

## 2

(a) a charge transport compound having the formula

(1)



where R<sub>1</sub> and R<sub>2</sub> are, independently, an (N,N-disubstituted)arylamine group, such as a julolidine group, a triphenyl amine group, or an N-substituted carbazole group;

R<sub>3</sub> and R<sub>4</sub> are, independently, an alkylsulfonylphenyl group; and

X is a linking group having the formula —(CH<sub>2</sub>)<sub>m</sub>—, branched or linear, where m is an integer between 0 and 20, inclusive, and one or more of the methylene groups is optionally replaced by an oxygen atom, a carbonyl group, urethane, urea, an ester group, a —NR<sub>5</sub> group, a CHR<sub>6</sub> group, or a CR<sub>7</sub>R<sub>8</sub> group where R<sub>5</sub>, R<sub>6</sub>, R<sub>7</sub>, and R<sub>8</sub> are, independently, H, an alkyl group, or aryl group;

(b) a charge generating compound; and

(c) an electrically conductive substrate over which the charge transport compound and the charge generating compound are located.

In a second aspect, the invention features an electrophotographic imaging apparatus that includes (a) a plurality of support rollers; and (b) the above-described organophotoreceptor operably connected to said support rollers with motion of the support rollers resulting in motion of said organophotoreceptor. The apparatus can further comprise a liquid or a dry toner dispenser.

In a third aspect, the invention features an electrophotographic imaging process that includes (a) applying an electrical charge to a surface of the above-described organophotoreceptor; (b) imagewise exposing the surface of the organophotoreceptor to radiation to dissipate charge in selected areas and thereby form a pattern of charged and uncharged areas on the surface; (c) contacting the surface with a toner, such as a liquid toner that includes a dispersion of colorant particles in an organic liquid, to create a toned image; and (d) transferring the toned image to a substrate.

In a fourth aspect, the invention features a novel charge transport material having the formula

(1)



where R<sub>1</sub> and R<sub>2</sub> are, independently, an (N,N-disubstituted)arylamine group, such as a julolidine group, a triphenyl amine group, or an N-substituted carbazole group;

R<sub>3</sub> and R<sub>4</sub> are, independently, an alkylsulfonylphenyl group; and

X is a linking group having the formula (CH<sub>2</sub>)<sub>m</sub>—, branched or linear, where m is an integer between 0 and 20, inclusive, and one or more of the methylene groups

is optionally replaced by an oxygen atom, a carbonyl group, urethane, urea, an ester group, a  $-\text{NR}_5$  group, a  $\text{CHR}_6$  group, or a  $\text{CR}_7\text{R}_8$  group where  $\text{R}_5$ ,  $\text{R}_6$ ,  $\text{R}_7$ , and  $\text{R}_8$  are, independently, H, an alkyl group, or aryl group.

These photoreceptors can be used successfully, for example, with liquid toners to produce high quality images. The high quality of the images can be maintained after repeated cycling.

Other features and advantages of the invention will be apparent from the following description of the preferred embodiments thereof, and from the claims.

#### DETAILED DESCRIPTION

Charge transport compounds with desirable properties can be formed having two linked sulfonylphenylhydrazone groups with the hydrazones having substitutions with an (N,N-disubstituted)arylamine groups or derivatives thereof. These charge transport compounds have desirable properties as evidenced by their performance in organophotoreceptors for electrophotography. The organophotoreceptors are particularly useful in laser printers and the like as well as photocopiers, scanners and other electronic devices based on electrophotography. The use of these charge transport compounds is described below in the context of laser printers use, although their application in other devices operating by electrophotography can be generalized from the discussion below.

To produce high quality images, particularly after multiple cycles, it is desirable for the charge transport compounds to form a homogeneous solution with the polymeric binder and remain approximately homogeneously distributed through the organophotoreceptor material during the cycling of the material. In addition, it is desirable to increase the amount of charge that the charge transport compounds can accept (indicated by a parameter known as the acceptance voltage or " $V_{acc}$ "), and to reduce retention of that charge upon discharge (indicated by a parameter known as the discharge voltage or " $V_{dis}$ ").

There are many charge transport compounds available for electrophotography. Examples of charge transport materials are pyrazoline derivatives, fluorene derivatives, oxadiazole derivatives, stilbene derivatives, hydrazone derivatives, carbazole hydrazone derivatives, polyvinyl carbazole, polyvinyl pyrene, or polyacenaphthylene. However, there is a need for other charge transport compounds to meet the various requirements of particular electrophotography applications.

In electrophotography applications, a charge generating compound within an organophotoreceptor absorbs light to form electron-hole pairs. These electron-hole pairs can be transported over an appropriate time frame under a large electric field to discharge locally a surface charge that is generating the field. The discharge of the field at a particular location results in a surface charge pattern that essentially matches the pattern drawn with the light. This charge pattern then can be used to guide toner deposition. The charge transport compounds described herein are especially effective at transporting charge, and in particular holes from the electron-hole pairs formed by the charge generating compound. In some embodiments, a specific electron transport compound can also be used along with the charge transport compound.

The layer or layers of materials containing the charge generating compound and the charge transport compounds are within an organophotoreceptor. To print a two dimensional image using the organophotoreceptor, the organophotoreceptor has a two dimensional surface for forming at least

a portion of the image. The imaging process then continues by cycling the organophotoreceptor to complete the formation of the entire image and/or for the processing of subsequent images.

5 The organophotoreceptor may be provided in the form of a plate, a flexible belt, a disk, a rigid drum, a sheet around a rigid or compliant drum, or the like. The charge transport compound can be in the same layer as the charge generating compound and/or in a different layer from the charge generating compound. Additional layers can be used also, as described further below.

10 In some embodiments, the organophotoreceptor material comprises, for example: (a) a charge transport layer comprising the charge transport compound and a polymeric binder, (b) a charge generating layer comprising the charge generating compound and a polymeric binder, and (c) the 15 electrically conductive substrate. The charge transport layer may be intermediate between the charge generating layer and the electrically conductive substrate. Alternatively, the charge generating layer may be intermediate between the charge transport layer and the electrically conductive substrate. 20 In further embodiments, the organophotoreceptor material has a single layer with both a charge transport compound and a charge generating compound within a polymeric binder.

25 The organophotoreceptors can be incorporated into an electrophotographic imaging apparatus, such as laser printers. In these devices, an image is formed from physical embodiments and converted to a light image that is scanned onto the organophotoreceptor to form a surface latent image. The surface latent image can be used to attract toner onto the 30 surface of the organophotoreceptor, in which the toned image is the same or the negative of the light image projected onto the organophotoreceptor. The toner can be a liquid toner or a dry toner. The toner is subsequently transferred, from the surface of the organophotoreceptor, to a receiving surface, such as a sheet of paper. After the 35 transfer of the toner, the entire surface is discharged, and the material is ready to cycle again. The imaging apparatus can further comprise, for example, a plurality of support rollers for transporting a paper receiving medium and/or for movement of the photoreceptor, suitable optics to form the light image, a light source, such as a laser, a toner source and 40 delivery system and an appropriate control system.

45 An electrophotographic imaging process generally can comprise (a) applying an electrical charge to a surface of the above-described organophotoreceptor; (b) imagewise exposing the surface of the organophotoreceptor to radiation 50 to dissipate charge in selected areas and thereby form a pattern of charged and uncharged areas on the surface; (c) exposing the surface with a toner, such as a liquid toner that includes a dispersion of colorant particles in an organic liquid to create a toned image, to attract toner to the charged or discharged regions of the organophotoreceptor, and (d) transferring the toned image to a substrate.

55 The improved charge transport compounds described herein comprises two sulphonylphenylhydrazone groups connected by a linking group and with an arylamine group substituted on each hydrazone group. Specifically, the improved charge transport compounds have the formula:



60 where X is the linking group,  $\text{R}_1$  and  $\text{R}_2$  are, independently, (N,N-disubstituted)arylamine groups and  $\text{R}_3$  and  $\text{R}_4$  are alkylsulfonylphenyl groups.

In describing chemicals by structural formulae and group definitions, certain terms are used in a nomenclature format that is chemically acceptable. The terms groups and moiety have specific meanings. The term group indicates that the generically recited chemical material (e.g., alkyl group, phenyl group, julolidine group, triphenyl amine group, carbazole group, alkylsulfonylphenyl group, etc.) may have any substituent thereon which is consistent with the bond structure of that group. For example, alkyl group includes alkyl materials such as methyl ethyl, propyl iso-octyl, dodecyl and the like, and also includes such substituted alkyls such as chloromethyl, dibromoethyl, 1,3-dicyanopropyl, 1,3,5-trihydroxyhexyl, 1,3,5-trifluorocyclohexyl, 1-methoxydodecyl, phenylpropyl and the like. However, as is consistent with such nomenclature, no substitution would be included within the term that would alter the fundamental bond structure of the underlying group. For example, where a phenyl group is recited, substitution such as 1-hydroxyphenyl, 2,4-fluorophenyl, orthocyanophenyl, 1,3,5-trimethoxyphenyl and the like would be acceptable within the terminology, while substitution of 1,1,2,2,3,3-hexamethylphenyl would not be acceptable as that substitution would require the ring bond structure of the phenyl group to be altered to a non-aromatic form because of the substitution. Where the term moiety is used, such as alkyl moiety or phenyl moiety, that terminology indicates that the chemical material is not substituted.

The charge transport compound may or may not be symmetrical. Thus, for example, R<sub>1</sub> and R<sub>2</sub> groups may be the same or different and R<sub>3</sub> and R<sub>4</sub> groups may be the same or different. In addition, the above-described formula for the charge transport compound is intended to cover isomers. Organophotoreceptors

The organophotoreceptor may be, for example, in the form of a plate, a flexible belt, a disk, a rigid drum, or a sheet around a rigid or compliant drum, with flexible belts and rigid drums generally being used in commercial embodiments. The organophotoreceptor may comprise, for example, an electrically conductive substrate and a photoconductive element in the form of one or more layers. The photoconductive element comprises both a charge transport compound and a charge generating compound in a polymeric binder, which may or may not be in the same layer. For example, in some embodiments with a single layer construction, the charge transport compound and the charge generating compound are in a single layer. In other embodiments, however, the photoconductive element comprises a bilayer construction featuring a charge generating layer and a separate charge transport layer. The charge generating layer may be located intermediate between the electrically conductive substrate and the charge transport layer. Alternatively, the photoconductive element may have a structure in which the charge transport layer is intermediate between the electrically conductive substrate and the charge generating layer. In the dual layer embodiments, the charge generation layer generally has a thickness from about 0.5 to about 2 microns, and the charge transport layer has a thickness from about 5 to about 35 microns. In a single layer embodiment, the layer with the charge generating compound and the charge transport compound generally has a thickness from about 7 to about 30 microns.

The electrically conductive substrate may be flexible, for example in the form of a flexible web or a belt, or inflexible, for example in the form of a drum. A drum can have a hollow cylindrical structure that provides for attachment of the drum to a drive that rotates the drum during the imaging process. Typically, a flexible electrically conductive sub-

strate comprises an electrically insulating substrate and a thin layer of electrically conductive material onto which the photoconductive material is applied.

The electrically insulating substrate may be paper or a film forming polymer such as polyethylene terephthalate, polyimide, polysulfone, polyethylene naphthalate, polypropylene, nylon, polyester, polycarbonate, polyvinyl fluoride, polystyrene and the like. Specific examples of polymers for supporting substrates included, for example, polyethersulfone (Stabar™ S-100, available from ICI), polyvinyl fluoride (Tedlar®, available from E.I. DuPont de Nemours & Company), polybisphenol-A polycarbonate (Makrofol™, available from Mobay Chemical Company) and amorphous polyethylene terephthalate (Melinar™, available from ICI Americas, Inc.). The electrically conductive materials may be graphite, dispersed carbon black, iodide, conductive polymers such as polypyroles and Calgon conductive polymer 261 (commercially available from Calgon Corporation, Inc., Pittsburgh, Pa.), metals such as aluminum, titanium, chromium, bras, gold, copper, palladium, nickel, or stainless steel, or metal oxide such as tin oxide or indium oxide. In embodiments of particular interest, the electrically conductive material is aluminum. Generally, the photoconductor substrate will have a thickness adequate to provide the required mechanical stability. For example, flexible web substrates generally have a thickness from about 0.01 to about 1 mm, while drum substrates generally have a thickness of from about 0.5 mm to about 2 mm.

The charge generating compound is a material which is capable of absorbing light to generate charge carriers, such as a dye or pigment. Examples of suitable charge generating compounds include metal-free phthalocyanines, metal phthalocyanines such as titanium phthalocyanine, copper phthalocyanine, oxytitanium phthalocyanine, hydroxygallium phthalocyanine, squarylium dyes and pigments, hydroxy-substituted squarylium pigments, perylimides, polynuclear quinones available from Allied Chemical Corporation under the tradename Indofast® Double Scarlet, Indofast® Violet Lake B, Indofast® Brilliant Scarlet and Indofast® Orange, quinacridones available from DuPont under the tradename Monastral™ Red, Monastral™ Violet and Monastral™ Red Y, naphthalene 1,4,5,8-tetracarboxylic acid derived pigments including the perinones, tetrabenzo-porphyrins and tetranaphthaloporphyrins, indigo- and thioindigo dyes, benzothioxanthene-derivatives, perylene 3,4,9,10-tetracarboxylic acid derived pigments, polyazopigments including bisazo-, trisazo- and tetrakisazo-pigments, polymethine dyes, dyes containing quinazoline groups, tertiary amines, amorphous selenium, selenium alloys such as selenium-tellurium, selenium-tellurium-arsenic and selenium-arsenic, cadmium sulphoselenide, cadmiumselenide, cadmium sulphide, and mixtures thereof. For some embodiments, the charge generating compound comprises oxytitanium phthalocyanine, hydroxygallium phthalocyanine or a combination thereof.

Generally, a charge generation layer comprises a binder in an amount from about 10 to about 90 weight percent and more preferably in an amount of from about 20 to about 75 weight percent, based on the weight of the charge generation layer. A charge transport layer generally comprises a binder in an amount from about 30 weight percent to about 70 weight percent. A single layer with a charge transport compound and a charge generating compound generally comprises a binder in an amount from about 10 weight percent to about 60 weight percent. A person of ordinary skill in the art will recognize that additional ranges of binder concentrations are contemplated and are within the present disclosure.

The binder generally is capable of dispersing or dissolving the charge transport compound (in the case of the charge transport layer or a single layer construction) and/or the charge generating compound (in the case of the charge generating layer or a single layer construction). Examples of suitable binders for both the charge generating layer and charge transport layer generally include, for example, polystyrene-co-butadiene, polystyrene-co-acrylonitrile, modified acrylic polymers, polyvinyl acetate, styrene-alkyd resins, soya-alkyl resins, polyvinylchloride, polyvinylidene chloride, polyacrylonitrile, polycarbonates, polyacrylic acid, polyacrylates, polymethacrylates, styrene polymers, polyvinyl butyral, alkyd resins, polyamides, polyurethanes, polyesters, polysulfones, polyethers, polyketones, phenoxy resins, epoxy resins, silicone resins, polysiloxanes, poly(hydroxyether) resins, polyhydroxystyrene resins, novolak, poly(phenylglycidyl ether)-co-dicyclopentadiene, copolymers of monomers used in the above-mentioned polymers and combinations thereof. Preferably, the binder is selected from the group consisting of polycarbonates, polyvinyl butyral, and a combination thereof. Examples of suitable polycarbonate binders include polycarbonate A which is derived from bisphenol-A, polycarbonate Z, which is derived from cyclohexylidene bisphenol, polycarbonate C, which is derived from methylbisphenol A, and polyester-carbonates. Examples of suitable of polyvinyl butyral are BX-1 and BX-5 form Sekisui Chemical Co. Ltd., Japan.

The photoreceptor may optionally have additional layers as well. Such additional layers can be, for example, a sub-layer and overcoat layers such as barrier layers, release layers, and adhesive layers. The release layer forms the uppermost layer of the photoconductor element. The barrier layer may be sandwiched between the release layer and the photoconductive element or used to overcoat the photoconductive element. The barrier layer provides protection from abrasion to the underlayers. The adhesive layer locates and improves the adhesion between the photoconductive element, the barrier layer and the release layer, or any combination thereof. The sub-layer is a charge blocking layer and locates between the electrically conductive substrate and the photoconductive element. The sub-layer may also improve the adhesion between the electrically conductive substrate and the photoconductive element.

Suitable barrier layers include, for example, coatings such as crosslinkable siloxanol-colloidal silica coating and hydroxylated silsesquioxane-colloidal silica coating, and organic binders such as polyvinyl alcohol, methyl vinyl ether/maleic anhydride copolymer, casein, polyvinyl pyrrolidone, polyacrylic acid, gelatin, starch, polyurethanes, polyimides, polyesters, polyamides, polyvinyl acetate, polyvinyl chloride, polyvinylidene chloride, polycarbonates, polyvinyl butyral, polyvinyl acetoacetal, polyvinyl formal, polyacrylonitrile, polymethyl methacrylate, polyacrylates, polyvinyl carbazoles, copolymers of monomers used in the above-mentioned polymers, vinyl chloride/vinyl acetate/vinyl alcohol terpolymers, vinyl chloride/vinyl acetate/maleic acid terpolymers, ethylene/vinyl acetate copolymers, vinyl chloride/vinylidene chloride copolymers, cellulose polymers, and mixtures thereof. The above barrier layer polymers optionally may contain small inorganic particles such as fumed silica, silica, titanic alumina, zirconia, or a

combination thereof. Barrier layers are described further in U.S. Pat. No. 6,001,522 to Woo et al., entitled "Barrier Layer For Photoconductor Elements Comprising An Organic Polymer And Silica," incorporated herein by reference. The release layer topcoat may comprise any release layer composition known in the art. In some embodiments, the release layer is a fluorinated polymer, siloxane polymer, fluorosilicone polymer, silane, polyethylene, polypropylene, polyacrylate, or a combination thereof. The release layers can comprise crosslinked polymers.

Generally, adhesive layers comprise a film forming polymer, such as polyester, polyvinylbutyral, polyvinylpyrrolidone, polyurethane, polymethyl methacrylate, poly(hydroxy amino ether) and the like.

Sub-layers can comprise, for example, polyvinylbutyral, organosilanes, hydrolyzable silanes, epoxy resins, polyesters, polyamides, polyurethanes, silicones and the like. In some embodiments, the sub-layer has a dry thickness between about 20 Angstroms and about 2,000 Angstroms. Sublayers containing metal oxide conductive particles can be 1-25 microns thick.

The charge transport compounds as described herein; and photoreceptors including these compounds, are suitable for use in an imaging process with either dry or liquid toner development. Liquid toner development can be desirable because it offers the advantages of providing higher resolution images and requiring lower energy for image fixing compared to dry toners. Examples of suitable liquid toners are known in the art. Liquid toners generally comprise toner particles dispersed in a carrier liquid. The toner particles can comprise a colorant/pigment, a resin binder, and/or a charge director. In some embodiments of liquid toner, a resin to pigment ratio can be from 2:1 to 10:1, and in other embodiments, from 4:1 to 8:1. Liquid toners are described further in Published U.S. Patent Applications 2002/0128349, entitled "Liquid Inks Comprising A Stable Organosol," 2002/0086916, entitled "Liquid Inks Comprising Treated Colorant Particles," and 2002/0197552, entitled "Phase Change Developer For Liquid Electrophotography," all three of which are incorporated herein by reference.

#### Charge Transport Compound

In some embodiments, the organophotoreceptors as described herein can comprise an improved charge transport compound with two sulfonylphenylhydrazone groups connected with a linker and with each hydrazone conjugated with an (N,N-disubstituted) arylamine group. The (N,N-disubstituted) arylamine groups comprise aromatic bonding within the structure with a nitrogen atom that is at least double substituted at the nitrogen atom. (N,N-disubstituted) arylamine groups of particular interest include, for example, a julolidine group, a triphenyl amine group, or an N-substituted carbazole group. Specifically, the compounds are based on a formula



**9**

where  $R_1$  and  $R_2$  are, independently, an (N,N-disubstituted)arylamine group, such as a julolidine group, a triphenyl amine group, or an N-substituted carbazole group;

$R_3$  and  $R_4$  are, independently, an alkylsulfonylphenyl group; and

X is a linking group having the formula  $-\text{CH}_2)_m-$ , branched or linear, where m is an integer between 0 and

**10**

20, inclusive, and one or more of the methylene groups is optionally replaced by an oxygen atom, a carbonyl group, urethane, urea, an ester group, a  $-\text{NR}_5$  group, a  $\text{CHR}_6$  group, or a  $\text{CR}_7\text{R}_8$  group where  $R_5$ ,  $R_6$ ,  $R_7$ , and  $R_8$  are, independently, H, an alkyl group, or aryl group.

Non-limiting examples of such charge transport compounds have the following formulas:



## 11

where R is  $\text{CH}_3(\text{CH}_2)_n$ —, branched or linear, where n is an integer between 0 and 30, inclusive,

(4)



These photoreceptors can be used successfully with liquid toners to produce high quality images. The high quality of the images can be maintained after repeated cycling.

#### Synthesis of Charge Transfer Compounds

Charge transport compounds can be synthesized from one or more hydrazone compounds along with a linking group, such as a dihalogenated compound. Each hydrazone compound can be formed from a hydrazine and an aldehyde or ketone with an N,N-disubstituted arylamine group. The hydrazines can be obtained commercially or synthesized.

The synthesis of the hydrazones can be performed with 4-methylsulfonylphenylhydrazine or derivatives thereof and an approximately molar equivalent of an aromatic aldehyde or aromatic ketone. 4-methylsulfonylphenylhydrazine hydrochloride is commercially available from Fisher Scientific, Pittsburgh, Pa. Various N,N-disubstituted arylamine aldehydes are available commercially or can be synthesized. Some representative examples are presented below.

Both 4-(diphenylamino)benzaldehyde and 9-ethyl-3-carbazolecarboxyaldehyde are available commercially from Aldrich, Milwaukee, Wis. Julolidine aldehyde can be synthesized from julolidine, which is available commercially from Aldrich, Milwaukee, Wis. Specifically, julolidine can be dissolved in warm N,N-dimethylformamide (DMF). After the julolidene is dissolved, the solution can be cooled. Then,  $\text{POCl}_3$  (10–15% excess) can be added slowly via a dropping funnel to the cooled DMF solution. After the addition of  $\text{POCl}_3$  was completed, the solution was heated over steam bath for a period of 1 hour then cooled to room temperature and added slowly to a large excess of water. The solid Julolidine aldehyde was filtered off and washed repeatedly with water. The product was dried at 50° C. vacuum oven for 4 hours.

The synthesis of the charge transport compounds from one or two hydrazones and a linking group can be performed

## 12

in an alkaline catalyzed reaction. Suitable linking groups are formed from halogenated, generally brominated, alkyl or substituted alkyl compounds. The reaction can be performed in a suitable solvent, for example, DMSO, to dissolve the hydrazone, optionally with heating. The mixture can then be heated, for example, at temperatures from 70° C. to 80° C. for four hours, to generate the reaction product. Then, the bishydrazone product can be cooled and purified.

To form an asymmetric charge transport compound with two different hydrazones, the reactions can be performed, for example, two different ways. In one embodiment, An excess amount of dibrominated linker group, generally at least in a molar ratio of two to one, is reacted with a first hydrazone. The product can be isolated as a solid and then reacted with the second hydrazone, for example, in a stoichiometric amount. In another embodiment, a linker with a bromine and a hydroxyl group is reacted with a first hydrazone. Then, the hydroxyl group is converted to a bromine group. A second hydrazone is reacted to the later formed bromine group to form a bishydrazone product with two different hydrazones.

A detailed procedure for the synthesis and characterization of compounds 2 and 4, as labeled above, is described in the Examples below. Compound 3 can be prepared according to the procedure for compound 2 except diphenylamino benzaldehyde is replaced by 9-ethyl-3-carbazolecarboxyaldehyde (available commercially from Aldrich Chemical Company).

#### Organophotoreceptor (OPR) Preparation Methods

Following conventional terminology, the number of layers in the OPR refers to the layers with charge transport compounds and/or charge generating compounds. Thus, the presence of overayers underlays, release layers and the like do not alter the single layer versus dual layer terminology.

#### Positive Inverted Dual Layer OPR

A positive polarity, inverted dual layer organic photoreceptor can be prepared by incorporating a charge transport compound disclosed herein into the charge transport layer and then over coating this layer with a charge generation solution to form a charge generation layer. The positive inverted dual layer is designed to operate with a positive surface charge that is discharge upon illumination at the point of illumination. An example of a specific approach for forming this structure is presented below.

In one embodiment, a charge transport solution comprising a 1:1 ratio by weight of a charge transport compound as described herein to a binder, such as polycarbonate Z; binder (commercially available from Mitsubishi Gas Chemical under the trade name Lupilon™ Z-200 resin), can be prepared by combining a solution of 1.25 g of one of the charge transport compounds as described herein in 8.0 g of tetrahydrofuran with 1.25 g of polycarbonate Z in 6.25 g of tetrahydrofuran. The charge transport solution can be hand coated onto a 76-micrometer (3-mil) thick aluminized polyester substrate (such as a Melinex® 442 polyester film from Dupont having a 1 ohm/square aluminum vapor coat) having a 0.3-micron polyester resin sub-layer (Vitel® PE-2200 from Bostik Findley, Middletown, Mass.). A knife coater, set to a 51-micrometer (2-mil) orifice between the blade and polyester, can be used to prepare a film with an 8–10-micron thickness after drying the wet film in an oven at 110° C. for 5–10 min.

13

A dispersion for forming a charge generation layer can be prepared by micronising 76.1 g of oxytitanium phthalocyanine pigment (H.W. Sands Corp., Jupiter, FL), 32.6 g of S-Lec B Bx-5 polyvinylbutyral resin (Sekisui Chemical Co. Ltd.), and 641.3 g of methyl ethyl ketone, using a horizontal sand mill operating in recycle mode for 8 hours. After milling, the charge generation layer base can be diluted with methyl ethyl ketone to decrease the total solids of the solution to 4.0 wt %. The charge generation solution can be hand-coated onto the charge transport layer using a knife coater, set to a 20–25 micron (0.8–1.0 mil) orifice between the blade and charge transport layer to prepare a sub-micron thick charge generation layer (CGL) film after drying the wet film in an oven at 110° C. for 3–5 min.

#### Negative Dual Layer OPR

A negative polarity, dual layer organic photoreceptor can be prepared forming a charge generation layer and then incorporating a charge transport compound disclosed herein into a solution and coating this solution over the charge generation layer to form a charge transport layer. A negative dual layer is designed to operate with a negative surface charge that is discharged upon illumination at the point of illumination. A specific example for forming a negative dual layer is described below.

In one embodiment, a charge generation layer mill-base dispersion can be prepared by micronising 76.1 g of oxytitanium phthalocyanine pigment, 32.6 g of S-Lec B Bx-5 polyvinylbutyral resin (Sekisui Chemical Co. Ltd.), and 641.3 g of methyl ethyl ketone, using a horizontal sand mill operating in recycle mode for 8 hours. Following milling the charge generating layer base can be diluted with methyl ethyl ketone to decrease the total solids of the solution to 4.0 wt %. The charge generation solution can be hand-coated onto a 76-micrometer (3-mil) thick aluminized polyester substrate (Melinex® 442 polyester film from Dupont having a 1 ohm/square aluminum vapor coat) having a 0.3-micron polyester resin sub-layer (Vitel® PE-2200 from Bostik Findley, Middletown, Mass.). A knife coater, set to a 20–25 micron (0.8–1.0 mil) orifice between the blade and substrate, can be used to prepare the sub-micron thick charge generating layer film after drying the wet film in an oven at 10° C. for 3–5 min.

A charge transport solution comprising a 1:1 ratio by weight of a charge transport compound described herein to polycarbonate Z binder is prepared by combining a solution of 125 g of the charge transport compound in 8.0 g of tetrahydrofuran with 1.25 g of polycarbonate Z in 6.25 g of tetrahydrofuran. A knife coater, set to a 51-micrometer (2-mil) orifice between the blade and polyester, can be used to prepare an 8–10-micron thick film after drying the wet film in an oven at 110° C. for 5–10 min.

#### Single Layer OPR

A single layer organic photoreceptor can be prepared by incorporating a charge transport compound disclosed herein along with a charge generating composition into a single coating solution and then coating this solution over a suitable substrate. A single layer OPR, in principle, can be designed to operate with a surface charge, which may be positive or negative, that is discharged upon illumination at the point of illumination in which the charge is generated in a layer and transported through that layer.

In practice, single layer OPRs are used predominantly with positive surface charges. In general, through the photoconductive and semiconductive materials of interest, electrons have a significantly lower mobility than holes. With low concentrations of charge generating pigment com-

14

pounds to limit charge trapping in a single layer structure, the electron-hole pairs can be generated some distance from the surface of the OPR after light is absorbed. However, the electron-hole pairs still tend to be closer to the surface than the substrate, such that the electron has less distance to travel than the hole in a positive single layer OPR. The hole from the electron-hole pair can transport through the remaining portion of the OPR to the underlying substrate. Thus, while electrons may travel some distance to neutralize positive charges at the surface of a positively charged OPR, the electrons would still have significantly larger distance to travel to the substrate in a negative single layer OPR. For single layer embodiments, it can be desirable to include an optional electron transport compound to facilitate the electron transport.

However, the use of a dual layer positive OPR is complicated by the formation of a thin charge generating layer over a charge transport layer due to processing complications of dip coating and solvent selection. Also, the thin charge generating layer can be abraded away in use without a good overcoat layer. Thus, a single layer positive OPR may offer some advantages over a positive dual layer system. Since the formation of negative dual layer OPRs do not have the complications of positive dual layer OPRs and since limited electron mobility hinders operation of negative single layer OPRs, negative single layer OPRs generally are less desirable although they are within the scope of the present disclosure for incorporation of the improved charge transport compounds described herein.

In one embodiment especially for the preparation of a single layer OPR, a charge transport pre-mix solution containing a 1:1 ratio by weight of a charge transport compound disclosed herein to polycarbonate Z binder can be prepared by combining a solution of 1.25 g of the charge transport compound in 8.0 g of tetrahydrofuran with 1.25 g of polycarbonate Z in 6.25 g of tetrahydrofuran. A charge generating layer mill-base dispersion can be prepared by micronising 76.1 g of oxytitanium phthalocyanine pigment, 32.6 g of polycarbonate Z binder resin, and 641.3 g of tetrahydrofuran, using a horizontal sand mill operating in pass mode for 68 passes. An electron transport pre-mix solution containing a 1:1.4 ratio of (4-n-butoxycarbonyl-9-fluorenylidene) malonitrile electron transport compound to Polycarbonate Z binder can be prepared by combining a solution of 1.25 g of one of the electron transporting material in 8.0 g of tetrahydrofuran with 1.75 g of polycarbonate Z in 9 g of tetrahydrofuran.

The single layer coating solution can be prepared by combining 14 g of the charge transport premix, 4.08 g of the electron transport premix and 1.92 g of the charge generating layer mill-base dispersion. The single layer solution can be hand-coated onto a 76 micrometer (3-mil) thick aluminized polyester substrate (Melinex® 442 polyester film from Dupont having a 1 ohm/square aluminum vapor coat) having a 0.3-micron polyester resin sub-layer (Vitel® PE-2200 from Bostik Findley, Middletown, Mass.). A knife coater, set to a 50–75 micron (2–3 mil) orifice between the blade and substrate, can be used to prepare a single layer film with an 8–10 micron thickness after drying the wet film in an oven at 110° C. for 5–10 min.

The invention will now be described further by way of the following examples.

#### EXAMPLES

##### Example 1

###### Synthesis And Characterization Charge Transport Compounds

This example described the synthesis and characterization of compounds 2 and 4, in which the numbers refer to

## 15

formula numbers above. The characterization involves both chemical characterization and the electronic characterization of materials formed with the compound.

## Compound 2

To a 2-liter 3-neck round bottom flask equipped with reflux condenser and mechanical stirrer were added 4(diphenylamino) benzaldehyde (112.0 g, 0.41 mole, commercially available from Aldrich, Milwaukee, Wis. and used as received) followed by the addition of 400 ml of tetrahydrofuran (THF). A mixture of 100 ml THF solution of 4+methylsulfonylphenylhydrazine hydrochloride (100 g, 0.45 mole, commercially obtained from Fisher Scientific, Pittsburgh, Pa.) was mixed with 66 g potassium carbonate (66 g, 0.5 mole) in 50 ml of water. The mixture was stirred for 0.5 hour and then was added to the 4-diphenylamino) benzaldehyde solution. The combined solution was refluxed for 2 hours. After cooled to room temperature, the corresponding hydrazone was obtained by evaporating the solvent.

To a 100 ml round bottom flask equipped with reflux condenser and magnetic stirrer were added the intermediate from the previous step (2.2 g, 5 mmol) and 1,5-dibromopentane (0.57 g, 2.5 mmol, obtained from Aldrich) and 50 ml of acetone. The mixture was stirred at room temperature until all solid entered into solution. Then KOH (1.12 g, 0.02 mol, obtained from Aldrich) was added into the reaction mixture. The reaction mixture was refluxed for 30 hours then cooled to room temperature and poured into water (100 ml). The aqueous solution was extracted with diethyl ether (3×50 ml). All ether solutions were combined and evaporated till 50 ml. The solid product separated out upon addition of the ether solution to 200 ml of hexane. The solid was filtered off and dried at 50° C. oven vacuum for 5 hours to obtain 1.02 g product (Yield=30.71%).

The product had a melting point of 97–97.5° C. The product was soluble in DMSO, toluene, THF, DMF, acetone, chloroform, and benzene. The proton NMR spectrum of the product had peaks that were interpreted as follows: <sup>1</sup>H NMR (Benzene):  $\delta$ =0.80–1.70 (m, 6H, —CH<sub>2</sub>—CH<sub>2</sub>—CH<sub>2</sub>—), 2.43 (s, 6H, CH<sub>3</sub>—S), 2.85 (m, 4H, —CH<sub>2</sub>—CH<sub>2</sub>—N), 6.80–7.95 (m, 36H, aromatic protons and 2H, Ar—CH=N—). The infrared spectrum of the product had peaks that were interpreted as follows: IR (KBr): 3010 (Ar), 2850–2750 (Al), 1580 (—C=N—), 1300 (—SO<sub>2</sub>—).

## Compound 4

Julolidine (173 g, 1 mole, obtained from Aldrich) was dissolved in N,N-dimethylformamide (DMF) (400 ml) then cooled in water bath to 5° C. POCl<sub>3</sub> (10–15% excess) was added slowly via a dropping funnel to the cooled DMF solution. After the addition of POCl<sub>3</sub> was completed, the solution was heated over steam bath for a period of 1 hour then cooled to room temperature and added slowly to a large excess of water. The solid Julolidine aldehyde was filtered off and washed repeatedly with water. The product was dried at 50° C. vacuum oven for 4 hours.

Julolidine aldehyde (82 g, 0.41 mole, prepared previously) was added to a 2-liter 3-neck round bottom flask equipped with reflux condenser and mechanical stirrer, followed by the addition of 400 ml of tetrahydrofuran (THF). A mixture of 100 ml THF solution of 4-methylsulfonylphenylhydrazine hydrochloride (100 g,

## 16

0.45 mole, commercially obtained from Fisher Scientific, Pittsburgh, Pa.) was mixed with 66 g potassium carbonate (66 g, 0.5 mole) in 50 ml of water, and the mixture was stirred for 0.5 hour. The mixture was then added to the Julolidine aldehyde solution. The combined solution was refluxed for 2 hours. After cooled to room temperature, the corresponding hydrazone was obtained by evaporating the solvent.

10 The intermediate from previous step (2.2 g, 6 mmol), 1,5-dibromopentane (0.70 g, 3 mmol, obtained from Aldrich) and 50 ml of DMF were added to a 100 ml round bottom flask equipped with reflux condenser and magnetic stirrer. The solution was stirred at room temperature until all solid 15 entered into solution. KOH (1.12 g, 0.02 mol) was added into the reaction mixture. The reaction mixture was refluxed for 24 hours, cooled to room temperature and poured into water. The product was filtered, dried, purified by column 20 chromatography (hexane/acetone: 3/1). The product obtained has a weight of 0.03 g for a yield of 6.25%.

The melting point of the product was 127–128° C. The product was soluble in DMSO, toluene, THF, DMF, acetone, chloroform, and benzene. The proton NMR spectrum had peaks that were interpreted as follows: <sup>1</sup>H NMR (Benzene):  $\delta$ =0.75–0.95 (p, 4H, —CH<sub>2</sub>—C<sub>2</sub>—CH<sub>2</sub>—), 1.05–1.30 (p, 8H, —CH<sub>2</sub>—CH<sub>2</sub>—CH<sub>2</sub>—), 1.48–1.72 (p, 2H, —CH<sub>2</sub>—CH<sub>2</sub>—CH<sub>2</sub>—), 2.40 (s, 6H, CH<sub>3</sub>—S), 2.45–2.85 (m, 8H, 25 —C—CH<sub>2</sub>—CH<sub>2</sub>— and 8H, —CH<sub>2</sub>—CH<sub>2</sub>—N), 3.00 (t, 2H, —CH<sub>2</sub>—CH<sub>2</sub>—N—), 3.30 (t, 2H, —CH<sub>2</sub>—CH<sub>2</sub>—N—), 6.80–7.85 (m, 14H, aromatic protons and 2H, Ar—CH=N—). The infrared spectrum of the product had peaks that were interpreted as follows: IR (KBr): 3010 (Aromatic), 2850–2750 (Aliphatic), 1580 (—C=N—), 1300 (—SO<sub>2</sub>—).

## Example 2

## Ionization Potential

This example provides measurements of the ionization potential for two-charge transport compounds synthesized as described in Example 1.

40 Samples for ionization potential (Ip) measurements were prepared by dissolving the compound in tetrahydrofuran. The solution was hand-coated on an aluminized polyester substrate that was precision coated with a methylcellulose-based adhesion sub-layer to form a charge transport material (CTM) layer. The role of this sub-layer was to improve adhesion of the CTM layer, to retard crystallization of CTM, and to eliminate the electron photoemission from the Al 45 layer through possible CTM layer defects. No photoemission was detected from the Al through the sub-layer at illumination with up to 6.4 eV quanta energy light. In addition, the adhesion sub-layer was conductive enough to avoid charge accumulation on it during measurement. The 50 thickness of both the sub-layer and CTM layer was ~0.4  $\mu$ m. No binder material was used with CTM in the preparation of 55 the samples for Ip measurements.

The ionization potential was measured by the electron photoemission in air method similar to that described in 60 “Ionization Potential of Organic Pigment Film by Atmospheric Photoelectron Emission Analysis”, *Electrophotography*, 28, Nr. 4, p. 364. (1989) by E. Miyamoto, Y.

Yamaguchi, and M. Yokoyama, which is hereby incorporated by reference. The samples were illuminated with monochromatic light from a quartz monochromator with a deuterium lamp source. The power of the incident light beam was  $2\text{--}5 \cdot 10^{-8}$  W. The negative voltage of  $-300$  V was supplied to the sample substrate. The counter-electrode with the  $4.5 \times 15 \text{ mm}^2$  slit for illumination was placed at 8 mm distance from the sample surface. The counterelectrode was connected to the input of the BK2-16 type electrometer, working in the open input regime, for the photocurrent measurement. A  $10^{15}\text{--}10^{12}$  amp photocurrent was flowing in the circuit under illumination. The photocurrent, I, was strongly dependent on the incident light photon energy  $h\nu$ . The  $I^{0.5} = f(h\nu)$  dependence was plotted. Usually the dependence of the square root of photocurrent on incident light quanta energy is well described by linear relationship near the threshold [see references "Ionization Potential of Organic Pigment Film by Atmospheric Photoelectron Emission Analysis", *Electrophotography*, 28, Nr. 4, p. 364. (1989) by E. Miyamoto, Y. Yamaguchi, and M. Yokoyama; and "Photoemission in Solids", Topics in Applied Physics, 26, 1-103. (1978) by M. Cordona and L. Ley, incorporated herein by reference]. The linear part of this dependence was extrapolated to the  $h\nu$  axis and  $I_p$  value: was determined as the photon energy at the interception point. The ionization potential measurement has an error of  $\pm 0.03$  eV.

The ionization potential data for compounds 2 and 4 are listed in Table 1.

TABLE 1

| Compound   | $\mu_0$<br>( $\text{cm}^2/\text{V} \cdot \text{s}$ ) | $\mu$ ( $\text{cm}^2/\text{V} \cdot \text{s}$ )<br>at $6.4 \cdot 10^5$<br>$\text{V}/\text{cm}$ | $\alpha$ ( $\text{cm}/\text{V}$ ) $^{0.5}$ | Ionization<br>Potential (eV) |
|------------|------------------------------------------------------|------------------------------------------------------------------------------------------------|--------------------------------------------|------------------------------|
| Compound 2 | $8.10^{-10}$                                         | $1.2 \cdot 10^{-7}$                                                                            | 0.0063                                     | 5.49                         |
| Compound 4 | $1.10^{-11}$                                         | $1.3 \cdot 10^{-8}$                                                                            | 0.0088                                     | 5.40                         |

## Example 3

## Hole Mobility

This example presents hole mobility measurements for the two charge transport compounds synthesized as described in Example 1.

The hole drift mobility was measured by a time of flight technique as described in "The discharge kinetics of negatively charged Se electrophotographic layers," Lithuanian Journal of Physics, 6, p. 569-576 (1966) by E. Montrimas, V. Gaidelis, and A. Pazera, which is hereby incorporated by reference. Positive corona charging created electric field inside the CTM layer. The charge carriers were generated at the layer surface by illumination with pulses of nitrogen laser (pulse duration was 2 ns, wavelength 337 nm). The layer surface potential decreased as a result of pulse illumination up to 1-5% of initial pre-illumination potential. The capacitance probe that was connected to the wide frequency band electrometer measured the speed of the surface potential  $dU/dt$ . The transit time  $t_p$  was determined by the change (kink) in the curve of the  $dU/dt$  transient in linear or double logarithmic scale. The drift mobility was calculated by the formula  $\mu = d^2/U_0 t_p$ , where  $d$  is the layer thickness and  $U_0$  is the surface potential at the moment of illumination.

To prepare the sample for the measurements, a mixture of 0.1 g of the charge transport compound and 0.1 g of polycarbonate Z 200 (S-LEC B BX-1, commercially obtained from Sekisui) was dissolved in 2 ml of THF. The solution was coated on the polyester film with conductive Al layer by the dip roller method. After drying for 1 h at  $80^\circ\text{C}$ , a clear 10  $\mu\text{m}$  thick layer was formed. Samples were

prepared for compounds 2 and 4. The hole mobility of the sample was measured and the results are presented in Table 1. Mobility values at electric field strength, E, of  $6.4\text{--}10^5$   $\text{V}/\text{cm}$  are given in the Table 1 along with zero field mobilities  $\mu_0$ . The mobility field dependencies may be approximated by the function

$$\mu \sim e^{\alpha \sqrt{E}}$$

where  $\alpha$  is parameter characterizing mobility field dependence. The value of the parameter:  $\alpha$  is also given in Table 1.

The embodiments above are intended to be illustrative and not limiting. Additional embodiments are within the claims. Although the present invention has been described with reference to particular embodiments, workers skilled in the art will recognize that changes may be made in form and detail without departing from the spirit and scope of the invention.

What is claimed is:

1. An organophotoreceptor comprising:

(a) a charge transport compound having the formula



where  $R_1$  and  $R_2$  are, independently, an (N,N-substituted) arylamine group;

$R_3$  and  $R_4$  are, independently, an alkylsulfonylphenyl group; and

X is a linking group having the formula  $-(\text{CH}_2)_m-$ , branched or linear, where  $m$  is an integer between 0 and 20, inclusive, and one or more of the methylene groups is optionally replaced by an oxygen atom, a carbonyl group, urethane, urea, an ester group, a  $-\text{NR}_5$  group, a  $\text{CHR}_6$  group, or a  $\text{CR}_7\text{R}_8$  group where  $\text{R}_5$ ,  $\text{R}_6$ ,  $\text{R}_7$ , and  $\text{R}_8$  are, independently, H, an alkyl group, or aryl group;

(b) a charge generating compound; and

(c) an electrically conductive substrate over which said charge transport compound and said charge generating compound are located.

2. An organophotoreceptor according to claim 1 wherein said organophotoreceptor is in the form of a flexible belt.

3. An organophotoreceptor according to claim 1 wherein said organophotoreceptor is in the form of a drum.

4. An organophotoreceptor according to claim 1 comprising:

(a) a charge transport layer comprising said charge transport compound and a polymeric binder; and

(b) a charge generating layer comprising said charge generating compound and a polymeric binder.

5. An organophotoreceptor according to claim 1 wherein said charge transport compound is selected from the group consisting of:



where R is  $\text{CH}_3(\text{CH}_2)_m$ , branched or linear, where n is an integer between 0 and 30, inclusive; and

21



6. An electrophotographic imaging apparatus comprising:  
 (a) a plurality of support rollers; and  
 (b) an organophotoreceptor operably connected to said support rollers with motion of the support rollers resulting in motion of said organophotoreceptor, said organophotoreceptor comprising:  
 (i) a charge transport compound having the formula



- where  $R_1$  and  $R_2$  are, independently, an (N,N-disubstituted)arylamine;  $R_3$  and  $R_4$  are, independently, an alkylsulfonylphenyl group; and  $X$  is a linking group having the formula  $-(CH_2)_m-$ , branched or linear, where  $m$  is an integer between 0 and 20, inclusive, and one or more of the methylene groups is optionally replaced by an oxygen atom, a carbonyl group, urethane, urea, an ester group, a  $-NR_5$  group, a  $CHR_6$  group, or a  $CR_7R_8$  group where  $R_5$ ,  $R_6$ ,  $R_7$ , and  $R_8$  are, independently, H, an alkyl group, or aryl group;  
 (ii) a charge generating compound; and  
 (iii) an electrically conductive substrate over which said charge transport compound and said charge generating compound are located.

7. The electrophotographic imaging apparatus of claim 6 wherein  $R_1$  and  $R_2$  are, independently, a julolidine group, a triphenyl amine group, or an N-substituted carbazole group.

8. The electrophotographic imaging apparatus of claim 6 further comprising a liquid toner dispenser.

9. The electrophotographic imaging apparatus of claim 6 wherein said organophotoreceptor comprises a drum that supports the electrically conductive substrate.

10. The electrophotographic imaging apparatus of claim 6 wherein said organophotoreceptor comprises a belt that supports the electrically conductive substrate.

11. An electrophotographic imaging process comprising:  
 (a) applying an electrical charge to a surface of an organophotoreceptor comprising:

22

- (i) a charge transport compound having the formula



where  $R_1$  and  $R_2$  are, independently, an (N,N-disubstituted)arylamine group;

$R_3$  and  $R_4$  are, independently, an alkylsulfonylphenyl group; and

$X$  is a linking group having the formula  $-(CH_2)_m-$ , branched or linear, where  $m$  is an integer between 0 and 20, inclusive, and one or more of the methylene groups is optionally replaced by an oxygen atom, a carbonyl group, urethane, urea, an ester group, a  $-NR_5$  group, a  $CHR_6$  group, or a  $CR_7R_8$  group where  $R_5$ ,  $R_6$ ,  $R_7$ , and  $R_8$  are, independently, H, an alkyl group, or aryl group;

(ii) a charge generating compound; and

(iii) an electrically conductive substrate over which said charge transport compound and said charge generating compound are located;

(b) imagewise exposing said surface of said organophotoreceptor to radiation to dissipate charge in selected areas and thereby form a pattern of charged and uncharged areas on said surface;

(c) contacting said surface with a liquid toner comprising a dispersion of colorant particles in an organic liquid to create a toned image; and

(d) transferring said toned image to a substrate.

12. The electrophotometric imaging process of claim 11 wherein  $R_1$  and  $R_2$  are, independently, a julolidine group, a triphenyl amine group, or a carbazole group.

13. A charge transport compound having the formula



where  $R_1$  and  $R_2$  are, independently, an (N,N-disubstituted)arylamine group;

$R_3$  and  $R_4$  are, independently, an alkylsulfonylphenyl group; and

$X$  is a linking group having the formula  $-(CH_2)_m-$ , branched or linear, where  $m$  is an integer between 0 and 20, inclusive, and one or more of the methylene groups is optionally replaced by an oxygen atom, a carbonyl group, urethane, urea, an ester group, a  $-NR_5$  group, a  $CHR_6$  group, or a  $CR_7R_8$  group where  $R_5$ ,  $R_6$ ,  $R_7$ , and  $R_8$  are, independently, H, an alkyl group, or aryl group.

14. The charge transport compound of claim 13 wherein  $R_1$  and  $R_2$  are, independently, a julolidine group, a triphenyl amine group, or a N-substituted carbazole group.

15. The charge transport compound of claim 13 wherein  $R_1$  and  $R_2$  each comprise a julolidine group.

16. The charge transport compound of claim 13 wherein  $R_1$  and  $R_2$  each comprise a triphenyl amine group.

17. The charge transport compound of claim 13 wherein  $R_1$  and  $R_2$  each comprise an N-substituted carbazole group.

18. The charge transport compound of claim 13 wherein  $R_1$  and  $R_2$  are different.

\* \* \* \* \*